

1

3,540,980

## PROCESS OF ROSIN SIZING PAPER

Harold L. Jones, Mobile, Ala., assignor to International Paper Company, New York, N.Y., a corporation of New York

No Drawing. Continuation of application Ser. No. 716,001, Mar. 26, 1968, which is a continuation-in-part of application Ser. No. 549,819, May 13, 1966. This application Oct. 30, 1968, Ser. No. 772,474

Int. Cl. D21d 3/00; D21h 3/34  
U.S. Cl. 162—180

6 Claims

## ABSTRACT OF THE DISCLOSURE

A process of sizing paper in which a water-soluble aluminate is added to aqueous wood pulp until its pH is at least 9, a material yielding hydrogen ions and non-aluminum-containing polyvalent anions is added to bring the pH down to not less than about 4.5, and rosin size is applied to the surface of paper made from the pulp.

This invention relates to the sizing of paper and to a novel method of increasing the resistance of paper to water penetration and otherwise enhancing the quality of the sizing of the paper.

This application is a continuation of S.N. 716,001, filed Mar. 26, 1968 now abandoned and a continuation-in-part of co-pending U.S. Ser. No. 549,819, filed May 13, 1966, now abandoned.

U.S. Pat. No. 3,074,843 issued to Lagally et al. shows a process of producing paper having high dry strength and good wet strength wherein aluminum hydroxide is precipitated by mixing an aluminum-containing compound and an acid, a base, or an aluminum salt in the absence of nonaluminum-containing polyvalent anions (e.g., the sulfate ion). Optimum results were achieved at a pH within the range of 6 to 9. See, particularly, column 6, lines 29 to 32, and column 2, lines 61 to 63, of the Lagally et al. patent. Lagally et al. stress their need to be free of nonaluminum-containing polyvalent anions by calling it essential to their invention. See column 2, lines 27 and 28, of the Lagally et al. patent.

It has now been found, however, that the stated need of Lagally et al. for the attainment of strength when wet can be obviated, and that remarkable levels of sizing can be obtained concurrently with the development of strength. It has been found that, if a water-soluble aluminate is added to an aqueous wood pulp slurry until its pH is at least 9, i.e., 9 or above and if a material yielding hydrogen ions such as sulfuric acid or papermaker's alum is then added to the pulp and aluminate mixture to bring the overall pH down, i.e., to bring the pH down to not less than about 4.5, aluminum hydroxide will precipitate in such a manner and to such a degree as to assure excellent levels of sizing once rosin size or the like is added to complete the process. In short, then, it has been found that, if the pH of the wood pulp is attended to correctly, the presence of the nonaluminum-containing polyvalent anions of papermaker's alum— $Al_2(SO_4)_3 \cdot 14H_2O$ —or sulfuric acid is of little or no deleterious effect. The following examples, which describe a standard sizing method (Example 1) and variations of the method of present invention (Examples 2 to 18), and tables, which compile data of tests made on products of the examples, confirm this finding:

## EXAMPLE 1

A mixture of 60% and 40% hardwood kraft pulp, bleached to 85% G.E. brightness, was refined in an

2

experimental beater, at 1.75% consistency, to 509 C.S. freeness. Forty grams (ovendry basis) of the refined pulp were suspended in distilled water at 3% consistency. Fortified size (commercially available Paper Product 2409) was added to the slurry at a rate of 42.8 pounds of size solids per ton of pulp. A mechanical stirrer was used to keep the slurry thoroughly mixed during the addition. Stirring was continued, and after five minutes papermaker's alum was added at the rate of 53.5 pounds  $Al_2(SO_4)_3 \cdot 14H_2O$  per ton of pulp. Stirring was continued for 10 minutes. pH of the slurry after the addition of alum was 4.0. A solution of half normal sodium hydroxide was added to pH 5.0. Stirring was continued for one minute. Consistency was adjusted to 0.375% with water containing enough hydrochloric acid to give pH 5.0. Handsheets were formed on a British sheet mold, pressed between a polished metal plate and blotters, clamped in rings, and dried in a forced-draft oven at 150° C. for 30 minutes. Basis weight and caliper averaged 100 pounds and 7.0 mils, respectively. Before testing, sheets were brought into equilibrium with the atmosphere of a room maintained at 50% relative humidity and 73° F.

## EXAMPLE 2

Thirty grams (ovendry basis) of the refined pulp used in Experiment 1 were adjusted to 3% consistency with distilled water. A solution of sodium aluminate (commercially available Nalco 680) was slowly added to the slurry at the rate of 90 pounds per ton of pulp. Stirring was rapid during this addition. After five minutes of continuous stirring, the slurry was transferred to a TAPPI standard disintegrator. The disintegrator was started, and as violent agitation began pH was adjusted to 5.5 by the addition of a normal solution of sulfuric acid. At this point, flocculation occurred. Cf., Curtman, L. J.; Qualitative Chemical Analysis; The MacMillan Company; New York, 1938; p. 181 and Kolthoff et al.; Textbook of Quantitative Inorganic Analysis (3rd ed.); The MacMillan Company; New York, 1952, p. 318. The slurry was returned to a beaker and stirring was continued for 25 minutes, during which period a solution of fortified rosin size (Paper Product 2409) was delivered into the mixture at the rate of 3.4 pounds of size solids per ton of pulp. The slurry was diluted to 0.375% consistency, and handsheets were prepared, pressed, and conditioned as in Experiment 1.

Each dried sheet was weighed, dipped in a solution of fortified rosin size (Paper Product 2409), blotted lightly, weighed, and heated to incipient dryness at 105° C. between a polished metal plate and blotters on a Carver press. The sized sheets were clamped in rings and dried in a forced-draft oven at 105° C. for 30 minutes. Size solids pickup was equivalent to 3.4 pounds per ton of pulp.

## EXAMPLE 3

Example 2 was repeated, except that the slurry of pulp and sodium aluminate was adjusted to pH 5.5 by the addition of a solution of papermaker's alum.

## EXAMPLE 4

Thirty grams (ovendry basis) of the pulp used in Experiment 1 were suspended in distilled water at 3% consistency. A solution of sodium aluminate was slowly added to the slurry at the rate of 90 pounds  $Na_2Al_2O_4 \cdot 3H_2O$  per ton of pulp. Stirring was rapid during this addition. The mixture was transferred to a TAPPI standard disintegrator, and as violent agitation began, a normal solution of sulfuric acid was rapidly added to the slurry in such volume as to lower pH to 5.5 and flocculation of the variety discussed in the Curtman

and Kolthoff et al. texts, supra, occurred. Agitation was continued for 30 seconds. The treated pulp was returned to a beaker and stirred at a moderate rate for 20 minutes. Handsheets were prepared, pressed, and dried as in Experiment 1. Each dried sheet was weighed, dipped in a fresh solution of fortified rosin size (Paper Product 2409), blotted lightly, weighed, and heated to incipient dryness at 105° C. between a polished metal plate and blotters on a Carver press. The sized sheets were clamped in rings and dried in a forced-draft oven at 105° C. for 30 minutes. Basis weight and caliper averaged 100 pounds and 7.0 mils, respectively. Size solid pickup was equivalent to 6.8 pounds per ton of pulp.

## EXAMPLE 5

Example 4 was repeated, except that pH of the slurry of pulp and sodium aluminate was adjusted to 5.5 by the addition of a solution of papermaker's alum.

## EXAMPLE 6

Thirty grams (ovendry basis) of the pulp used in Experiment 1 were suspended in distilled water at 3% consistency. A solution of sodium aluminate was slowly added to the slurry at the rate of 90 pounds  $\text{Na}_2\text{Al}_2\text{O}_4 \cdot 3\text{H}_2\text{O}$  per ton of pulp. Stirring was rapid during this addition. While stirring continued, 0.5 N sulfuric acid was slowly added in such volume as to lower pH to 5.5 and flocculation of the variety discussed in the Curtman and Kolthoff et al. texts, supra, occurred. Agitation was continued for 20 minutes. Handsheets were prepared, pressed, and dried as in Experiment 1. Each dried sheet was weighed, dipped in a fresh solution of fortified rosin size (Paper Product 2409), blotted lightly, weighed, and heated to incipient dryness at 105° C. between polished metal plates and blotters on a Carver press. The sized sheets were clamped in rings and dried in a forced-draft oven at 105° C. for 30 minutes. Basis weight and caliper averaged 100 pounds and 7.0 mils, respectively. Size solids pickup was equivalent to 6.8 pounds per ton of pulp.

## EXAMPLE 7

Example 6 was repeated, except that pH of the slurry of pulp and sodium aluminate was adjusted to 5.5 by the addition of a solution of papermaker's alum.

## EXAMPLE 8

Example 6 was repeated, except that sodium aluminate was used at the rate of 60 pounds per ton of pulp, and that size solids pickup was equivalent to 15 pounds per ton of pulp.

## EXAMPLE 9

Example 8 was repeated, except that pH of the slurry of pulp and sodium aluminate was adjusted to 5.5 by the addition of a solution of papermaker's alum.

## EXAMPLE 10

Thirty grams (ovendry basis) of the refined pulp used in Experiment 1 were adjusted to 3% consistency with distilled water. A solution of sodium aluminate was slowly added to the slurry at the rate of 90 pounds  $\text{Na}_2\text{Al}_2\text{O}_4 \cdot 3\text{H}_2\text{O}$  per ton of pulp. Stirring was rapid during this addition. The mixture was transferred to a TAPPI standard disintegrator. The disintegrator was started, and as violent agitation began, 0.5 normal sulfuric acid was rapidly added to the slurry in such volume as to lower pH to 5.5. Here, flocculation as discussed in the Curtman and Kolthoff et al. texts, supra, occurred. Violent agitation was continued for 30 seconds; the treated pulp was returned to a beaker and stirred at a moderate rate for 20 minutes. Handsheets were prepared, pressed, and dried as in Experiment 1. Each dried sheet was weighed, dipped in a fresh solution of pale rosin size (Paper Product 2408A), blotted lightly, weighed, and heated to incipient

dryness at 105° C. between a polished metal plate and blotters on a Carver press. The sized sheets were clamped in rings and dried in a forced-draft oven at 105° C. for 30 minutes. Basis weight and caliper averaged 100 pounds and 7.0 mils respectively. Size solids pickup was equivalent to 5.7 pounds per ton of pulp.

## EXAMPLE 11

Example 10 was repeated, except that pH of the slurry of pulp and sodium aluminate was adjusted to 5.5 by the addition of a solution of papermaker's alum.

## EXAMPLE 12

Example 4 was repeated, except that the pulp was unbleached pine kraft, and that pH of the slurry of pulp and sodium aluminate was adjusted to 5.5 by the addition of 0.5 N sulfuric acid.

## EXAMPLE 13

Example 12 was repeated, except that pH of the slurry of pulp and sodium aluminate was adjusted to 5.5 by the addition of a solution of papermaker's alum.

## EXAMPLE 14

Four hundred thirty grams of pulp (ovendry basis) similar to that used in Experiment 1 were weighed into a Valley beater and diluted to 1.75% consistency with demineralized water. A solution of sodium aluminate containing the equivalent of 90 pounds  $\text{Na}_2\text{Al}_2\text{O}_4 \cdot 3\text{H}_2\text{O}$  per ton of pulp was added to the slurry during mixing. A 0.5 N solution of sulfuric acid was added to adjust pH to 5.5. Here, flocculation as discussed in the Curtman and Kolthoff et al. texts, supra, occurred. Mixing was continued for 20 minutes after the addition of acid before refining was begun. With a 5-kilogram weight in place, the pulp was beaten for 21 minutes to 509 C.S. freeness. The refined pulp was transferred to a large container and diluted with demineralized water (at pH 5.5) to sheetmaking consistency. Handsheets were prepared, pressed, dried, sized, and conditioned as in Experiment 4.

## EXAMPLE 15

Example 8 was repeated, except that a solution of sodium aluminate containing the equivalent of 40 pounds  $\text{Na}_2\text{Al}_2\text{O}_4 \cdot 3\text{H}_2\text{O}$  per ton of pulp was added to the slurry during mixing.

## EXAMPLE 16

Example 15 was repeated, except that pH of the slurry of pulp and sodium aluminate was adjusted to 5.5 by the addition of a solution of papermaker's alum.

## EXAMPLE 17

Example 15 was repeated, except that pH of the slurry of pulp and sodium aluminate was adjusted to 6.5 by the addition of a 0.5 N solution of sulfuric acid.

## EXAMPLE 18

Example 17 was repeated, except that pH of the slurry of pulp and sodium aluminate was adjusted to 4.5 by the addition of a 0.5 N solution of sulfuric acid.

## EXAMPLE 19

Thirty grams (ovendry basis) of bleached kraft pulp at C.S. freeness 500 were suspended in distilled water at 3% consistency. A solution of sodium aluminate was slowly added to the slurry at the rate of 90 pounds  $\text{Na}_2\text{Al}_2\text{O}_4 \cdot 3\text{H}_2\text{O}$  per ton of pulp. Stirring was rapid during this addition. While stirring continued, a normal solution of orthophosphoric acid was slowly added in such volume as to lower pH to 5.4 and flocculation of the variety discussed in the Curtman and Kolthoff et al. texts, supra, occurred. Agitation was continued for 20 minutes. Handsheets were prepared, pressed, and dried as in Experiment 1. Each dried sheet was weighed, dipped in a

fresh solution of fortified rosin size (Paper Product 2409), blotted lightly, weighed, and heated to incipient dryness at 105° C. between polished metal plates and blotters on a Carver press. The sized sheets were clamped in rings and dried in a forced-draft oven at 105° C. for 30 minutes. Basis weight and caliper averaged 100 pounds and 7.0 mils, respectively. Size solids pickup was equivalent to 6.8 pounds per ton of pulp.

#### EXAMPLE 20

Forty grams (ovendry basis) of refined pulp similar to that used in Example 1 were suspended in distilled water at 3% consistency. Slurry pH was adjusted to 1.9 by the slow addition of a normal solution of sulfuric acid. Stirring was rapid during this addition. After five minutes of continuous stirring, the slurry was transferred to a TAPPI standard disintegrator. The disintegrator was started, and as violent agitation began pH was adjusted to 5.5 by the addition of a solution of sodium aluminate at the rate of 90 pounds per ton of pulp. Flocculation occurred.

The slurry was returned to a beaker and stirring was continued for 25 minutes, during which period a solution of fortified rosin size was delivered into the mixture at the rate of 3.4 pounds of size solids per ton of pulp. The slurry was diluted to 0.375% consistency, and handsheets were prepared, pressed, and conditioned as in Example 1.

Each dried sheet was weighed, dipped in a solution of fortified rosin size, blotted lightly, weighed, and heated to incipient dryness at 105° C. between a polished metal plate and blotters on a Pasadena press. The sized sheets were clamped in rings and dried in a forced-draft oven at 105° C. for 30 minutes. Size solids pickup was equivalent to 3.4 pounds per ton of pulp.

#### EXAMPLE 21

Forty grams (ovendry basis) of pulp similar to that used in Example 1 were suspended in distilled water at 3% consistency. Slurry pH was adjusted to 1.9 by the addition of a normal solution of sulfuric acid. Stirring was rapid after this addition. The mixture was transferred to a TAPPI standard disintegrator and as violent agitation began a solution of sodium aluminate was added in such volume as to lower pH to 5.5. Flocculation occurred.

Agitation was continued for 30 seconds. The treated pulp was returned to a beaker and stirred at a moderate rate for 20 minutes. Handsheets were prepared, pressed, and dried as in Example 1. Each dried sheet was weighed, dipped in a fresh solution of fortified rosin size, blotted lightly, weighed, and heated to incipient dryness at 105° C. between a polished metal plate and blotters on a Pasadena press. The sized sheets were clamped in rings and dried in a forced-draft oven at 105° C. for 30 minutes. Basis weight and caliper averaged 100 pounds and 7.0 mils, respectively. Size solids pickup was equivalent to 6.8 pounds per ton of pulp.

#### EXAMPLE 22

Example 21 was repeated, except that pH of the pulp slurry was adjusted to 3.7 by the addition of a solution of papermaker's alum before adding a solution of sodium aluminate to flocculation pH 5.5.

#### EXAMPLE 23

Forty grams (ovendry basis) of pulp similar to that used in Example 1 were suspended in distilled water at 3% consistency. While the slurry was slowly stirred, pH was adjusted to 1.9 by the slow addition of half normal sulfuric acid. After 5 minutes pH was adjusted to 5.5 by the addition of a solution of sodium aluminate containing the equivalent of 90 pounds Na<sub>2</sub>Al<sub>2</sub>O<sub>4</sub>·3H<sub>2</sub>O per ton of pulp. Agitation was continued for 20 minutes. Handsheets were prepared, pressed, and dried as in Example 1. Each dried sheet was weighed, dipped in a fresh solution

of fortified rosin size, blotted lightly, weighed, and heated to incipient dryness at 105° C. between polished metal plates and blotters on a Pasadena press. The sized sheets were clamped in rings and dried in a forced-draft oven at 105° C. for 30 minutes. Basis weight and caliper average 100 pounds and 7.0 mils, respectively. Size solids pickup was equivalent to 6.8 pounds per ton of pulp.

#### EXAMPLE 24

Example 23 was repeated, except that sulfuric acid was added to the pulp slurry in such amount that flocculation pH 5.5 was attained by the addition of the equivalent of 60 pounds Na<sub>2</sub>Al<sub>2</sub>O<sub>4</sub>·3H<sub>2</sub>O per ton of pulp.

#### EXAMPLE 25

Example 24 was repeated, except that the volume of sulfuric acid used to adjust slurry pH was such as to require only 40 pounds Na<sub>2</sub>Al<sub>2</sub>O<sub>4</sub>·3H<sub>2</sub>O per ton of pulp to give flocculation pH 5.5.

20 TABLE 1

|             | Lactic acid<br>pene-<br>scope,<br>minutes | Coffee<br>pene-<br>scope,<br>minutes | Dry<br>indi-<br>cator,<br>seconds | Cobb<br>size, g./<br>sq. m. | Water<br>absorp-<br>tion,<br>percent |
|-------------|-------------------------------------------|--------------------------------------|-----------------------------------|-----------------------------|--------------------------------------|
| 25 Example: |                                           |                                      |                                   |                             |                                      |
| 1           | 1.7                                       | 21                                   | 131                               | 38                          | 60                                   |
| 2           | 6.8                                       | 90+                                  | 131                               | 29                          | 56                                   |
| 3           | 6.9                                       | 90+                                  | 119                               | 32                          | 53                                   |
| 4           | 13                                        | 90+                                  | 131                               | 30                          | 53                                   |
| 5           | 19                                        | 90+                                  | 119                               | 32                          | 52                                   |
| 6           | 23                                        | 90+                                  | 135                               | 31                          | 53                                   |
| 7           | 38                                        | 90+                                  | 138                               | 28                          | 49                                   |
| 8           | 49                                        | 90+                                  | 148                               | 26                          | 49                                   |
| 9           | 15                                        | 90+                                  | 156                               | 27                          | 51                                   |
| 10          | 18                                        | 90+                                  | 128                               | 29                          | 61                                   |
| 11          | 13                                        | 90+                                  | 109                               | 32                          | 59                                   |
| 12          | 34                                        | 26                                   | 137                               | 28                          | 46                                   |
| 13          | 30                                        | 90+                                  | 133                               | 28                          | 44                                   |
| 14          | 15                                        | 90+                                  | 128                               | 27                          | 49                                   |
| 15          | 20                                        | 19                                   | 152                               | 27                          | 49                                   |
| 16          | 23                                        | 90+                                  | 155                               | 28                          | 48                                   |
| 17          | 22                                        | 7.0                                  | 155                               | 26                          | 53                                   |
| 18          | 16                                        | 17                                   | 156                               | 26                          | 49                                   |
| 19          | 23                                        | 5                                    | 173                               | 39                          | 53                                   |
| 20          | 5.6                                       | 24                                   | 154                               | 28                          | 62                                   |
| 21          | 58                                        | 90+                                  | 157                               | 28                          | 56                                   |
| 22          | 20                                        | 90+                                  | 142                               | 30                          | 53                                   |
| 23          | 31                                        | 66                                   | 161                               | 29                          | 58                                   |
| 24          | 128                                       | 60                                   | 174                               | 26                          | 55                                   |
| 25          | 93                                        | 33                                   | 212                               | 28                          | 57                                   |

The data set forth in Table I, supra, suggest that a unique and remarkably effective method of sizing paper has been developed. Sizing by the present flocculated aluminate-rosin size procedure has produced handsheets superior in the characteristics evaluated to similar sheets prepared by orthodox means.

45 The following additional observations are worthy of note:

Variations in flocculation pH between 4.5 and 6.5 have little influence on sizing (Examples 15, 17, and 18, Table I);

55 Violent agitation during and immediately after flocculation does not appear to affect sizing (Examples 4 and 6, Table I); and

Both fortified rosin size and regular pale rosin size are compatible with the flocculated aluminate system (Examples 2 and 10, Table I).

60 What is claimed is:

1. A process for sizing paper made from wood pulp comprising a step of adding a water-soluble aluminate to an aqueous slurry of wood pulp in an amount sufficient to bring the pH of the aqueous slurry of the wood pulp to about 9 and above, a step of adding a material yielding hydrogen ions and non-aluminum-containing polyvalent anions to the aqueous slurry of wood pulp in an amount sufficient to flocculate the aluminate without lowering the pH of the aqueous slurry of the wood pulp beyond about 4.5, and a step of adding a rosin size to the wood pulp after it is transformed from the aqueous slurry into a web of paper.

2. A process for sizing paper made from wood pulp comprising a first step of adding a water-soluble aluminate

to an aqueous slurry of wood pulp in an amount sufficient to bring the pH of the aqueous slurry of wood pulp to about 9 and above, a second step of adding a material yielding hydrogen ions and non-aluminum-containing polyvalent anions to the aqueous slurry of wood pulp in an amount sufficient to flocculate the aluminate without lowering the pH of the aqueous slurry of the wood pulp beyond about 4.5, and a third step of adding a rosin size to the wood pulp after it is transformed from the aqueous slurry into a web of paper.

3. The process of claim 1 wherein the water-soluble aluminate is sodium aluminate.

4. The process of claim 1 wherein the material is sulfuric acid.

5. The process of claim 1 wherein the material is paper-  
maker's alum.

6. The process of claim 1 wherein a portion of the rosin size is added to the aqueous slurry of the wood pulp.

#### References Cited

##### UNITED STATES PATENTS

1,300,357 4/1919 De Cew ----- 162—180  
3,421,976 1/1969 Jones ----- 162—185

10 S. LEON BASHORE, Primary Examiner

R. H. ANDERSON, Assistant Examiner

U.S. Cl. X.R.

15 162—181, 183, 185